

## UNITED STATES PATENT OFFICE

2,234,363

## PROCESS OF IMPREGNATING FIBROUS MATERIAL AND THE MATERIAL THUS OBTAINED

Arnold Brunner and Georg von Finck, Frankfort-on-the-Main, Germany, assignors to I. G. Farbenindustrie Aktiengesellschaft, Frankfort-on-the-Main, Germany

No Drawing. Application January 8, 1938, Serial No. 184,104. In Germany January 13, 1937

12 Claims. (Cl. 91—70)

The present invention relates to a process of treating artificial or natural materials, such as fibers, yarns, ribbons, threads, textile fabrics and similar materials and to the material thus obtained. It is an object of our invention to treat the said materials with one or more impregnating agents for improving their properties. It is a further object of our invention to impart water-repellent properties to the said materials.

10 As materials to be treated according to the present invention various products come into question, especially such as are obtained from cellulose fibers, such as cotton, viscose artificial silk, cuprammonium artificial silk, products from cellulose esters or cellulose ethers and products from animal fibers such as wool and silk. There may also be used mixed yarns or mixed fabrics from the above materials, for instance, half-wool or mixtures from wool and artificial silk staple fiber. Many other fibrous materials may, furthermore, be used, for instance, flax, hemp, jute, ramie. These materials may, according to the process of the present invention, be rendered water-repellent.

25 Water-proofing impregnations are known. For instance, there are obtained by treatment with paraffin and salts of alumina textile materials from which the water immediately runs off in drops. This water-proofing effect is, however, lost when the material is washed but once. It has already been proposed to treat textiles with solutions in organic media, or with emulsions, of derivatives of fatty acids of high molecular weight, for instance fatty acid anhydrides or chlorides and thereby to make the textile water-repellent.

30 We have found that textile materials may be made water-repellent, with a very good success, by treating them with a solution or an emulsion of the substances obtainable according to the co-pending application Serial No. 168,681 filed October 12, 1937, now U. S. Patent No. 2,180,791, dated November 21, 1939, a division of application Serial No. 128,025 filed February 26, 1937, now U. S. Patent No. 2,165,956, dated July 11, 1939, in the name of Arnold Brunner, for "Condensation products and a process of preparing them."

The products to be used for the impregnation may be made as follows:

35 Phenols containing in the nucleus one or more aliphatic chains having at least 4 carbon atoms are treated with aqueous formaldehyde solutions and hydrogen chloride. The chloromethyl derivatives of the phenols thus formed having the formula  $A\text{CH}_2\text{Cl}$ , wherein A represents a radical of a phenol substituted by aliphatic hydrocarbon

radicals having at least 4 carbon atoms are caused to react with organic nitrogen bases, especially tertiary organic nitrogen bases, such as pyridine, triethylamine or the like, the corresponding quaternary ammonium compounds being obtained in the latter case. By the impregnation with the above-named compounds the textile goods are rendered waterproof so that they can be wetted by water only with difficulty. Other impregnating or finishing agents may further be added to the solution.

40 A great advantage of the invention resides in the fact that even after repeated washing with soap and sodium carbonate or benzine the material does not lose its water-repellent effect. Moreover, it is a great simplification that aqueous solutions or emulsions of the treating agent may be used for the impregnation.

The above indicated fibrous materials, for instance, yarns or fabrics, are impregnated, at ordinary or elevated temperature, with aqueous solutions or emulsions of the above-mentioned nitrogen containing compounds. The excess of liquid is removed by squeezing or centrifuging and the material is then dried, preferably at an elevated temperature. The drying operation may also be performed at lower temperatures, the dry material being then exposed to higher temperatures.

45 Instead of aqueous solutions or emulsions there may also be used solutions in organic solvents or the treating agent may be applied to the fibrous material, without using any solvent or diluent, at ordinary or elevated temperature. It is, however, most preferable to work in aqueous solutions or emulsions.

The following examples serve to illustrate the invention, but they are not intended to limit it thereto; the parts are by weight:

50 (1) 10 parts of the pyridinium compound obtained from the chloromethyl compound of the commercial mixture of isododecyl-, isotridecyl- and isotetradecyl-phenol are dissolved in 1000 parts of water. A fabric of cotton or viscose artificial silk is impregnated with this solution, dried at 110° C. and subsequently washed with soap and sodium carbonate or benzine.

55 (2) 10 parts of the quaternary ammonium compound obtained from the chloromethyl compound of isododecyl-phenol and triethylamine are dissolved in 1000 parts of water. Wool or half-wool is impregnated with this solution at 60° C. and

dried at 140° C. A good water-repellent effect is obtained which is stable to washing.

(3) The impregnating agent is prepared in the following way:

5 Hydrogen chloride is led, for 15 hours, at 15° C. into a mixture of 160 parts of dodecyl-phenol, 120 parts of strong hydrochloric acid and 80 parts of para-formaldehyde. The resin-like product formed is separated from the mother liquor; it contains 12.9 per cent. of chlorine.

10 62 parts of this product are dissolved in 100 parts of alcohol and 22 parts of methyl-aniline are added thereto. After a one hour's heating under reflux, such an amount of alcohol is added that 15 a solution of about 10 per cent. strength is obtained.

15 50 parts of this solution are poured into 950 parts of water. Cotton or acetate artificial silk is impregnated with the liquid and dried at 140° C.

20 The material has properties similar to those of the fibrous material which has been treated as described in Example 1.

(4) By substituting in Example 3 for the 950 parts of water the corresponding quantity of alcohol and impregnating the material with this 25 solution, a similar effect is obtained.

(5) 5 parts of the pyridinium compound obtainable from chloromethyl-iso-octylphenol are dissolved in 1000 parts of water and the solution is 30 used for impregnating cotton, viscose artificial silk or silk. After drying at 80° C. the material has a good water-repellent effect.

(6) Dress-goods from a mixture of wool and artificial silk staple fiber (50:50), from cotton, 35 viscose artificial silk or acetate artificial silk or natural silk are impregnated with a solution containing per liter of water 15 grams of a condensation product from chloromethyl-isobutyl-phenol and trimethyl-amine, squeezed and, after drying 40 at 60° C.-80° C. heated, for 20 minutes at 130° C. The material thus treated, especially light-weight artificial silk fabric, has been imparted, besides water-repellent properties, a good non-slip finish.

(7) Stuff for water-proofs from wool, cotton or 45 artificial silk is treated, for 5 minutes, with a solution containing 20 grams of a condensation product from pyridine and chloromethyl-diethyl-phenol, centrifuged and dried at 110° C.-120° C.

(8) A fabric from half-wool or half-silk is 50 treated, for 15 minutes, with a solution containing per liter of alcohol 10 grams of a condensation product from pyridine and chloromethyl-n-dodecyl-phenol, squeezed, dried and subsequently heated, for 15 minutes, at 140° C.

55 Instead of chloromethyl-n-dodecyl-phenol, there may also be used chloromethyl-iso-dodecyl-phenol.

We claim:

1. The process which comprises impregnating 60 fibrous materials with organic nitrogen compounds obtained by causing phenols of the general formula  $A.CH_2.Cl$ , wherein A represents a radical of a phenol substituted by aliphatic hydrocarbon radicals having a least 4 carbon atoms, to react 65 with a nitrogen base selected from the group consisting of tertiary aliphatic and tertiary heterocyclic amines and subsequently heating the impregnated material.

2. The process which comprises impregnating 70 fibrous materials with organic nitrogen compounds obtained by causing phenols of the general formula  $A.CH_2.Cl$ , wherein A represents a radical of a phenol substituted by one aliphatic hydro-

carbon radical having at least 4 carbon atoms, to react with a nitrogen base selected from the group consisting of tertiary aliphatic and tertiary heterocyclic amines and subsequently heating the impregnated material.

3. The process which comprises impregnating fibrous materials with organic nitrogen compounds obtained by causing phenols of the general formula  $A.CH_2.Cl$ , wherein A represents a radical of a phenol substituted by aliphatic hydrocarbon 10 radicals having at least 4 carbon atoms, to react with pyridine and subsequently heating the impregnated material.

4. The process of water-proofing textile materials which comprises impregnating textile materials with the compound obtained by condensation of pyridine and the chloromethyl compound of the commercial mixture of isododecyl-, isotri-decyl- and isotetradecyl-phenol and subsequently 15 heating the impregnated material.

5. The process of water-proofing textile materials which comprises impregnating textile materials with the compound obtained by condensation of pyridine and the chloromethyl compound of isododecyl-phenol and subsequently 20 heating the impregnated material.

6. The process of water-proofing textile materials which comprises impregnating textile materials with the compound obtained by condensation of pyridine and the chloromethyl compound 30 of isoctyl-phenol and subsequently heating the impregnated material.

7. Water-proof fibrous material which has been impregnated with organic nitrogen compounds obtained by causing phenols of the general formula  $A.CH_2.Cl$ , wherein A represents a radical of a phenol substituted by aliphatic hydrocarbon radicals having at least 4 carbon atoms, to react 35 with a nitrogen base selected from the group consisting of tertiary aliphatic and tertiary heterocyclic amines.

8. Water-proof fibrous material which has been impregnated with organic nitrogen compounds obtained by causing phenols of the general formula  $A.CH_2.Cl$ , wherein A represents a radical of a phenol substituted by one aliphatic hydrocarbon radical having at least 4 carbon atoms, to react 45 with a nitrogen base selected from the group consisting of tertiary aliphatic and tertiary heterocyclic amines.

9. Water-proof fibrous material which has been impregnated with organic nitrogen compounds obtained by causing phenols of the general formula  $A.CH_2.Cl$ , wherein A represents a radical of a phenol substituted by aliphatic hydrocarbon 55 radicals having at least 4 carbon atoms, to react with pyridine.

10. Water-proof textile material which has been impregnated with the compound obtained by condensation of pyridine and the chloromethyl compound of the commercial mixture of iso-dodecyl-, iso-tridecyl- and iso-tetradecyl-phenol.

11. Water-proof textile material which has been impregnated with the compound obtained by condensation of pyridine and the chloromethyl compound of isododecyl-phenol.

12. Water-proof textile material which has been impregnated with the compound obtained by condensation of pyridine and the chloromethyl compound of iso-octyl-phenol.